

1

2,861,894

## COAL TAR SOFT PITCH PRODUCT

Heinz Franck, Duisburg-Meiderich, Germany, assignor to  
Gesellschaft fuer Teerverwertung m. b. H., Duisburg-  
Meiderich, Germany, a corporation of Germany

No Drawing. Application July 5, 1955  
Serial No. 520,110

Claims priority, application Germany July 5, 1954

8 Claims. (Cl. 106—279)

The invention relates to a coal tar soft pitch product 15 and to a process for the manufacture thereof, and also to mixtures of this coal tar soft pitch with distilled bitu-

5

10

components takes place differ slightly; for instance, separation into the components tar and bitumen usually takes place at a bitumen content of about 20%. Therefore, to exclude as far as possible separation into the components, a bitumen content of 15% of a bitumen of the type B45 is prescribed for road tars with a bitumen additive by the German Industrial Standards regarding bituminous binders for road construction (DIN 1995).

However, it is of considerable practical interest to provide compositions of bitumen and tar of unlimited miscibility, when using types of bitumen such as they are mentioned in DIN 1995, namely bitumen of the types B15, B45, B65, B80, B200 and B300, because a bitumen content of 15%, as set forth in DIN 1995, is too low to appreciably affect the properties of the soft pitch contained in the bitumen tars. Such different types of bitumen possess the following properties:

|         | Type of bitumen |        |       |       |       |       |     |
|---------|-----------------|--------|-------|-------|-------|-------|-----|
|         | B300            | B200   | B80   | B65   | B45   | B25   | B15 |
| 250-320 | 160-210         | 70-100 | 50-70 | 35-50 | 20-30 | 10-20 |     |
| 27-37   | 37-44           | 44-49  | 49-54 | 54-59 | 59-67 | 67-72 |     |
| 16-24   | 24-30           | 30-35  | 35-40 | 40-45 | 45-53 | 53-58 |     |
| -20     | -15             | -10    | -8    | -6    | -2    | +3    |     |
| 0.5     | 0.5             | 0.5    | 0.5   | 0.5   | 0.5   | 0.5   |     |
| 0.5     | 0.5             | 0.5    | 0.5   | 0.5   | 0.5   | 0.5   |     |
| 100     |                 |        |       |       |       |       |     |
| 2.0     | 2.0             | 2.0    | 2.0   | 2.0   | 1.5   | 2.0   | 5   |
| 0.99    | 1.0             | 1.0    | 1.0   | 1.0   | 1.0   | 1.0   | 1.0 |
| 2.5     | 2.0             | 1.5    | 1.0   | 1.0   | 1.0   | 1.0   | 1.0 |
| 10      | 10              | 10     | 10    | 10    | 10    | 10    | 10  |
| -15     | -10             | -8     | -6    | -5    | ±0    | +5    |     |
| 60      | 60              | 60     | 60    | 60    | 60    | 50    | 40  |
| 50      |                 |        |       |       |       |       |     |
|         | 50              | 50     | 50    | 15    | 5     | 2     |     |

men. The term "distilled bitumen" as used hereinafter in the specification and in the claims designates the bituminous residue of normal petroleum distillation.

It is one object of the present invention to provide a coal tar soft pitch product which is miscible homogeneously and in practically any proportion with distilled bitumen and even with relatively soft bitumen.

The miscibility of tar with distilled bitumen is limited. It is known that bitumen with a high softening point which has been oxidized or distilled under a high vacuum can be mixed in any desired proportion with coal tar (see British Patent No. 506,677). However, only small amounts of tar can be mixed with large amounts of a bitumen which has not been previously treated in a special manner, i. e. with distilled bitumen. Only such a distilled bitumen is of interest for practical purposes, while bitumen with a high melting point which has been oxidized or distilled under a high vacuum is only of minor industrial importance. On the other hand large amounts of tar can also be homogeneously be mixed with small amounts of bitumen. Thus, homogeneous miscibility between tar and distilled bitumen in those proportions which are of industrial interest does not exist. Depending on the type of bitumen and tar used, the bitumen contents at which separation into the

45 Heretofore, however, it was not possible to increase the bitumen content of such tar-bitumen compositions. Consequently, even recently it was necessary to issue warnings against road tar compositions containing blended bitumen or soft bitumen, since failures in road construction projects have occurred when such mixtures were used. Such failures were due to the separation of the tar-bitumen mixtures into their components which had taken place (see, for instance H. Mallison, V. f. T.-Mitteilungen, "Strassenbau und Bautenschutz mit Steinkohlensteer," 1953, Issue 1, page 8).

50 It has now been found that a tar product homogeneously miscible in any proportion with distilled bitumen and even with relatively soft bitumen, i. e. a soft pitch product, is produced by mixing a coal tar pitch with a softening point (according to Krämer-Sarnow) of 60-80° C. with a tar oil fraction which consists essentially of a mixture of quadrinuclear aromatic coal tar components. Such quadrinuclear aromatic substances are, for instance, chrysene, pyrene, fluoranthene, naphthacene, and others. Such tar oil fractions are, for instance, disclosed in "Brennstoffchemie," vol. 1953, page 38, and vol. 1955, pages 14 to 16. The resulting mixture of a coal tar pitch with a softening point between 60° C. and 80° C. and preferably with a softening point of 70° C. and a coal

tar oil fraction consisting essentially of quadrinuclear aromatic coal tar components in an amount sufficient to reduce the softening point of the soft pitch product to below about 40° C., which mixture represents an important object of the present invention, is homogeneously miscible with any type of distilled bitumen.

If a coal tar pitch is mixed according to the present invention with such an amount of a tar oil fraction consisting essentially of quadrinuclear aromatic coal tar components that the softening point of the resulting mixture is lowered to below 40° C., a soft pitch product is formed which is compatible in any proportion, i. e. which is homogeneously miscible, with the bituminous residue of a standard petroleum distillation process known to the art as distilled bitumen, such as medium-hard bitumen, for instance, of the type B45, and even softer types.

It is another object of the present invention to provide such a composition of a mixture of the new soft pitch product and a distilled bitumen which composition is useful in road construction.

The tar oil fraction used for preparing the soft pitch product according to the present invention is preferably free of substances which precipitate in crystalline form on mixing with the coal tar pitch. A tar oil fraction is therefore used in which its constituents are in eutectic equilibrium. The eutectic equilibrium may, if necessary, be produced by thoroughly cooling the oil and removing by centrifuging the crystallized solid substance.

The coal tar pitch to be employed according to the invention is preferably a pitch which has been obtained by continuous distillation under gentle thermal conditions (see, for instance, H. J. Winkler "Der Steinkohlen-tre und seine Aufarbeitung," Essen, 1951, pages 21-24). It is also possible to use a pitch obtained by intermittent distillation. However, coal tar pitch obtained by distillation under cracking conditions should not be used, since the compatibility of such a coal tar pitch with distilled bitumen is the more diminished, the higher its content of cracking residues (soot-like compounds of high molecular weight).

The soft pitch product according to the invention can be mixed with the distilled bitumen without any special precaution and in any desired proportion.

According to a further preferred form of the present invention a small amount of an oil with a high phenol content is added to the mixture of soft pitch product and bitumen. It has been found that the properties of the mixture of soft pitch product and bitumen are favorably affected if 1% to 6% and preferably about 2% of an oil rich in phenols, for instance, an oil prepared according to the process disclosed in German Patent No. 807,689, is added thereto. Such a preferred tar oil rich in phenol is produced, for instance, by distillation of equal parts of phenol pitch, i. e. the residue remaining on working up crude phenol by distillation, and anthracene oil until the residue has the softening point of a normal pitch.

As stated hereinabove any desired type of bitumen may be used for the purpose of the present invention. Advantageously a bitumen with a penetration value of 35-50 (100 g., 5 seconds, 25° C.) and preferably with a density higher than 1.03 at 20° C. is used. However, types of bitumen with a lower density are also suitable.

The pitch-bitumen mixture according to the present invention, prepared by using a soft pitch product according to this invention, is suitable for all the purposes for which pitch or bitumen or mixtures thereof are used.

The composition according to the present invention may be used as such or in mixture with light coal tar oils and may thus be adjusted to the viscosity of road tar or of blended bitumen.

If a mixture of equal amounts of coal tar pitch (softening point 60-80° C.), bitumen (B45), and a tar oil fraction consisting essentially of quadrinuclear aromatic coal tar components in an amount sufficient to reduce

the softening point (according to Kraemer-Sarnow) of the mixture to a softening point below 30° C. is used for the production of a tar-bitumen binder of low viscosity, and if a fluxing oil is added thereto, there is obtained a binding agent which combines the advantages of road tar and blended bitumen. In addition, such a composition is homogeneously miscible in any proportion with road tar as well as with blended bitumen.

What I claim is:

1. Soft pitch product homogeneously miscible in all proportions with distilled bitumen, said pitch product consisting essentially of a mixture of coal tar pitch with a softening point of about 70° C., and a coal tar oil fraction consisting essentially of quadrinuclear aromatic coal tar components, said soft pitch product having a softening point lower than about 40° C.
2. The mixture of distilled bitumen and a soft pitch product in all proportions, said soft pitch product consisting essentially of a mixture of coal tar pitch with a softening point between about 60° C. and about 80° C., and a coal tar oil fraction consisting essentially of quadrinuclear aromatic coal tar components, said soft pitch product having a softening point lower than about 40° C.
3. The mixture of distilled bitumen and a soft pitch product in all proportions, said soft pitch product consisting essentially of a mixture of coal tar pitch with a softening point of about 70° C., and a coal tar oil fraction consisting essentially of quadrinuclear aromatic coal tar components, said soft pitch product having a softening point lower than about 40° C.
4. The mixture of distilled bitumen and a soft pitch product in all proportions, said soft pitch product consisting essentially of a mixture of coal tar pitch with a softening point between about 60° C. and about 80° C., and a coal tar oil fraction consisting essentially of quadrinuclear aromatic coal tar components, said soft pitch product having a softening point lower than about 40° C., said bitumen-pitch mixture containing between about 1% and about 6% of an oil rich in high boiling and high molecular phenols.

5. The mixture of distilled bitumen and a soft pitch product in all proportions, said soft pitch product consisting essentially of a mixture of coal tar pitch with a softening point between about 60° C. and about 80° C., and a coal tar oil fraction consisting essentially of quadrinuclear aromatic coal tar components, said soft pitch product having a softening point lower than about 40° C., said bitumen-pitch mixture containing about 2% of an oil rich in high boiling and high molecular phenols.

6. In a process of producing a soft pitch product homogeneously miscible with bituminous distillation residues of the petroleum distillation in all proportions, the step comprising intimately mixing coal tar pitch with a soft point between about 60° C. and about 80° C. with a coal tar oil fraction consisting essentially of quadrinuclear aromatic coal tar components, said coal tar oil fraction being added in an amount sufficient to decrease the softening point of the resulting soft pitch product below about 40° C.

7. Bituminous road surfacing material comprising a mixture of about equal parts of the bituminous distillation residue of the petroleum distillation and the soft pitch product consisting essentially of a mixture of coal tar pitch with a softening point of about 70° C., and a coal tar oil fraction consisting essentially of quadrinuclear aromatic coal tar components, said soft pitch product having a softening point lower than about 40° C., and a diluting tar oil added to said mixture of bituminous distillation residue and soft pitch product in an amount sufficient to impart to said mixture the viscosity of road tar.

8. Soft pitch product having a softening point lower than about 40° C. and being homogeneously miscible with distilled bitumen in all proportions, said soft pitch

product consisting essentially of a mixture of coal tar pitch with a softening point of 60-80° C., and a coal tar oil fraction consisting essentially of quadrinuclear aromatic coal tar components, said coal tar oil fraction being admixed to said coal tar pitch in an amount sufficient to decrease the softening point of said coal tar pitch to a softening point lower than about 40° C.

References Cited in the file of this patent

UNITED STATES PATENTS

701,743 Lee June 3, 1902

924,086  
1,970,164  
2,123,560  
2,131,085  
5 2,395,853

216,245  
358,974  
363,698  
538,308  
601,784

Meadows et al. ----- June 8, 1909  
Breuer ----- Aug. 14, 1934  
Bennett ----- July 12, 1938  
Anderton ----- Sept. 27, 1938  
Fair ----- Mar. 5, 1946

FOREIGN PATENTS

Great Britain ----- May 29, 1924  
Great Britain ----- Oct. 12, 1931  
Great Britain ----- Dec. 21, 1931  
Great Britain ----- July 29, 1941  
Great Britain ----- May 12, 1948